

## UNITED STATES PATENT OFFICE.

EMILE THEODORE JOSEPH WATREMEZ, OF AVILLY, PAR SENLIS, FRANCE.

## PROCESS FOR SCOURING VEGETABLE FIBERS, &amp;c.

1,370,076.

Specification of Letters Patent.

Patented Mar. 1, 1921.

No Drawing.

Application filed October 29, 1919. Serial No. 334,345.

*To all whom it may concern:*

Be it known that I, EMILE THEODORE JOSEPH WATREMEZ, citizen of the Republic of France, and resident of Avilly, par 5 Senlis, Oise, France, have invented a new and useful Process for Scouring Vegetable Fibers, &c., which improvements are fully set forth in the following specification.

The process according to the present invention is based on the use in scouring baths consisting essentially in a mixture of alkali or alkaline salt, metallic oxid and a hypochlorite such as Javelle water. The metallic oxid may be replaced if desired, by the 10 metal itself reduced to powder. Any metal may be employed, preferably zinc.

It should be understood that the proportions of the various constituents of the bath may be varied.

20 By way of example, for the treatment of cotton fibers the following proportions are preferably used:—

Caustic soda lye of 30° to 35°

25 Baumé strength \_\_\_\_\_ 40 liters  
Javelle water of commercial strength viz. 16° to 18° Baumé 30 liters  
Into this solution is stirred, in the cold, zinc oxid \_\_\_\_\_ 1 kilog.

30 After two hours stirring, sufficient water is added to make the total volume up to 1000 liters.

The fibers to be treated are steeped with the bath liquor by means of pressure rollers.

35 As soon as they are uniformly steeped, they are preferably placed in a keir into which the bath liquor is pumped until the fibers are completely covered.

The fibers are kept immersed in the bath 40 during a period of 12 to 24 hours and even longer, the time varying with the nature of the product.

The characteristic feature of the bath as described above consists in its composition, 45 that is to say the mixture of an alkali-metal hypochlorite and a salt of an alkali metal.

The treatment of the fibers with these products if used separately and not in conjunction in the same bath would not give any satisfactory result.

When the fibers are lifted from the bath they are rinsed and at once placed in an acid bath consisting, for example of two 50 parts per thousand (by volume) of sulfuric

acid of 60° Baumé strength, which is heated nearly to boiling point.

The fibers are treated for several minutes and are then rinsed again, being afterward subjected to the bleaching process proper. 60

In certain cases the action of the original bath is so powerful that no subsequent bleaching is necessary, the fibers after the second above-mentioned rinsing, being sufficiently bleached for industrial use. 65

When the fibers are very difficult to scour and bleach the operation may be repeated several times without any danger to the fibers, with or without a bleaching operation between two consecutive scourings, that is 70 to say, for instance, on leaving the acid bath the fibers are treated with a hypochlorite in the ordinary apparatus and are then returned to the original bath. The fibers may be passed through the original 75 bath several times.

If instead of working in the cold it is preferred to treat the fibers in a boiling hot bath, the composition of the bath may be modified as follows:— 80

The bath is prepared by treating the metallic oxid, or better still, a metal in the pulverized state, either simultaneously with an alkali or an alkali-metal hypochlorite, and a soluble reducing salt such as a 85 thiosulfate, a sulfite, or a hydrosulfite, or successively with the hypochlorite and a reducing salt on the one hand, and the alkali on the other hand. In this latter case the alkali is added to the already existing mixture. 90

By way of example, if zinc is utilized as the reducing metal the following proportions may be used for treating 1000 kilogs. of material:—

Sodium thiosulfate ( $Na_2S_2O_3$ ) 25 kilogs. is dissolved in commercial Javelle water 50 liters. Zinc powder 5 kilogs. is then stirred into the solution, which is left standing for 12 hours. Caustic soda lye of 30° Baumé 100 150 liters is added and after stirring, the mixture is left standing for 24 hours.

The unattacked zinc particles rapidly subside after agitation of the mass which is decanted but should not be filtered. In 105 this way a mixture is obtained of entirely different appearance and properties from that obtained by simply treating the metal with an alkali.

These proportions and qualities may of 110

course be varied according to the nature of the fibers to be treated and the effect which it is desired to obtain.

This mixture is diluted with water in order to bring the bath to the desired volume and is then heated to boiling point.

The bath has a tendency to become neutral by reason of the intense action on the natural coloring matters. It is necessary to 10 watch it and to add, if necessary, caustic soda in small quantities, in order to maintain the alkalinity.

Boiling is prolonged for 4 to 6 hours.

Then, in order to attain a still more complete scouring, the combined substances existing in the fiber are precipitated by adding 15 kilogs. of slaked lime and by continuing the boiling for 3 to 4 hours.

It should be noted that on the one hand 20 the complete removal of the precipitated substances is indispensable and that on the other hand, the compounds with ammonia as the base are the most easily attacked.

Before the acid treatment described below, 25 the fibers are immersed for 2 to 3 hours in a bath containing, for example 5 to 7 per cent., by volume, of ammonium sulfate. After rinsing they are immersed for 2 to 4 hours in a cold acid bath consisting 30 for instance of 2 per cent. by volume of sulfuric acid of 60° Baumé strength.

Thereupon the fiber is rinsed and is then ready for rapid and complete bleaching by the ordinary means.

35 The bath is so effective that in certain cases the operation can even be performed in the cold, but in such case it is preferable to pass the fiber after a summary rinsing, through milk of lime. This allows the first 40 bath to be preserved, all that is necessary being to replenish it.

The immersion in the milk of lime bath 45 may be sufficient when operating in the cold, the treatment with an ammoniacal salt and with acid being effected in the above-described manner.

It should be remarked that the precipitation with lime and the subsequent elimination by an ammoniacal salt and an acid can

be applied to any treatment based on the use of a soluble salt of an alkali-metal salt in order to effect the scouring.

I claim as my invention:

1. A process for scouring fibers of vegetable origin with the object of facilitating and accelerating their final bleaching, characterized by the feature that the fibers to be treated are immersed in the cold in a bath consisting of a mixture of an alkali, a metallic oxid and an alkali metal hypochlorite, for a time varying from 12 to 24 hours, thereupon rinsed, treated in the warm for several minutes with sulfuric acid solution and finally rinsed.

2. A process of scouring vegetable fibers, 65 consisting in steeping the fibers in a bath comprising an alkali, a metallic substance and an alkali-metal hypochlorite; then successively rinsing the fibers, treating them with sulfuric acid solution and again rinsing them.

3. A process of scouring vegetable fibers, consisting in steeping the fibers in a bath comprising an alkali, Javelle water and zinc; and then successively rinsing the 75 fibers, treating them with sulfuric acid solution and again rinsing them.

4. A process of scouring vegetable fibers, consisting in steeping the fibers in a bath comprising an alkali, Javelle water and 80 zinc; and then rinsing the fibers.

5. The herein-disclosed process of scouring vegetable fibers, which consists in dissolving a soluble alkali metal hypochlorite in a soluble alkaline reducing salt, and then 85 subjecting a metal to the action of the solution thus obtained; then steeping the fibers in the solution obtained from the action of the first solution on the metal; and then rinsing the fibers.

In testimony whereof I have signed this specification in the presence of two subscribing witnesses.

EMILE THEODORE JOSEPH WATREMEZ.

Witnesses:

PICOCOR,  
CHAS. P. PRESSLY.